

Feb. 5, 1952

C. B. ALLER

2,584,317

METHOD OF PRODUCING BIMETALLIC PRINTING FORMS

Filed Dec. 29, 1947

Fig.1.



Fig.2.



Fig.3.



Fig.4.



INVENTOR  
CLAES BØRGE ALLER

BY *Sol Shapiro*  
ATTORNEY

## UNITED STATES PATENT OFFICE

2,584,317

## METHOD OF PRODUCING BIMETALLIC PRINTING FORMS

Claes Børge Aller, Copenhagen, Denmark

Application December 29, 1947, Serial No. 794,257  
In Denmark September 9, 1946Section 1, Public Law 690, August 8, 1946  
Patent expires September 9, 1966

2 Claims. (Cl. 204—17)

**1.** The present invention relates to a method of producing bimetallic printing forms, i. e. printing forms in which the parts of the printing surface which are to transfer ink during printing are made of another metal than the parts that are not required to transfer ink. Bimetallic printing forms are mostly used for planographic printing, particularly offset, the two metals being so chosen that in presence of water one will retain the water and repel ink whereas the other one in spite of the presence of water will retain printer's ink and thus transfer ink in the printing process. In such planographic printing processes the height of the ink-retaining parts may differ from that of the ink-repelling parts of the printing plate, but in most cases there is either no difference in height or the difference is so small that it is of no significance for printing purposes. The present invention more particularly relates to the production of printing plates of the latter kind.

In the production of such planographic printing plates it is known to deposit on the surface of the metal which is to form one of the surface components in the printing process a continuous layer of the metal which is to form the other surface component after which a copying layer is applied to the surface of the metallic layer last mentioned, after which copying is carried out and the copying layer is developed, and the parts of the metallic intermediate layer which are not covered by the copying layer after development are etched right through to the supporting layer. In order to better protect the parts of the intermediate metallic layer covered by the parts of the copy remaining after development the latter may be hardened by being "burnt in" or by "melting in" suitable protecting agents. After etching said protecting agents and the parts of the copying layer not removed in development may be removed in known manner.

This known method suffers from several drawbacks. Thus it has been found that there cannot be obtained in this manner a true recording and a sufficient protection of the finer printing elements during etching. This is due to the etching agent being to some extent capable of penetrating to the back of the protecting layer from the borders of the areas protected and thus alter the size or shape of the printing elements or cause them to adhere insufficiently to the support and thus detach themselves.

It is also known to deposit the ink-retaining metal component through the openings of a copy produced directly on the surface of the other

metal component. In this process it has, however, been difficult to obtain a deposit of equal thickness in smaller and greater printing areas. Consequently in many cases a correct recording of the values of halftones cannot be obtained and the printing elements will in some places wear too fast or detach.

Moreover it has been proposed in a method which allegedly can be used in connection with both relief, intaglio and planographic printing to deep-etch the supporting metal after areas of another metal, "filling-in" metal, have been deposited thereon through the openings of a copy as described above, using for the said deep-etching an etching agent which does not attack the filling-in metal. In order to broaden the base part of the said filling-in metal to make it adhere better to the support a layer of resin is applied between the supporting and the copying layer and after development of the copy the resin is removed within the non-covered areas the removal being extended slightly behind the covered areas too in order to allow for the said broadening of the base of the filling-in metal. This method, however, is not suited for planographic plates, since the said base will alter the value of the half tones.

The object of this invention is a method of producing planographic printing forms in which all these drawbacks are removed. Other objects and purposes of the invention will appear from the following description and claims.

Broadly the invention consists in a method of producing planographic printing forms in which a protecting image is used for protecting the parts of the printing surface of the form which are not to be attacked by the etching agent during etching and the feature characterizing the invention is that the protecting image is applied to the surface of a galvanically deposited thin continuous intermediate layer of a metal acting as one of the metallic components in the planographic printing process, which intermediate metal layer is again placed upon a base layer of a material acting as the other metallic component in the bimetallic planographic printing process, and the non-protected parts of the metallic intermediate layer are etched away right through to the surface of the base metal by an etching agent which does not attack the protecting metal.

More particularly according to the invention the method is applied to the production of printing forms in which one of the components entering in the bimetallic printing process is chro-

mium or a chromium-containing alloy or stainless steel.

Between the intermediate layer and the protecting metal and between the intermediate layer and the base metal which layers are both of metals forming the components of a bimetallic planographic printing process there may be interposed other metals for instance silver for other purposes such as for improving adhesion or facilitating good deposition. The claims are to be understood so as to comprise methods in which this is the case if for any purpose it should be desired.

In contradistinction to the known method in which a continuous metal layer deposited on a support of the metal which is to form one of the components in a bimetallic printing process is protected during etching by a copy, a metal is used according to the present invention for the protection of the areas which are not to be attacked during etching, which has the effect that these parts will not at all be attacked. Consequently recording will be exact and the printing elements will not alter their size or shape or adhere insufficiently to the support.

The method which forms the subject matter of the present invention moreover differs from the known method in which the one metallic component is deposited upon the other one through the openings of a copy placed thereon in that none of the two metallic components in the bimetallic planographic printing process are according to the present invention deposited through the openings of the copy. Thereby it is avoided that the deposited metallic component of the said process will appear in undesired unevenness of thickness.

From the known method which is also mentioned above in which the base metal is deep-etched after a metal has been deposited on it through the openings of a copy produced on the surface thereof the present method differs not only in that no resin layer is interposed between the base metal and the copy as mentioned above but also in that the metallic intermediate layer that is interposed between the base and the copy is so thin that a deep etching cannot be carried out thereon without etching right through it and in that the said intermediate layer forms one of the metallic components and the base metal the other component of the bimetallic planographic printing process proper. In the etching there will be laid free areas of this base metal corresponding in size and shape exactly to the original copy. The exactness is due to the thinness of the intermediate layer and the capability of the protecting layer to completely protect the parts covered thereby. Such exactness will not be obtained in the known method even if etching is carried to such a depth that it reaches a further base plate supporting the first one and being of steel. This appears from the fact that the walls of the pits produced by etching are not vertical and that the purpose of the resinous layer used in the known method is to avoid the walls being vertical in order to secure the parts remaining after etching a broader base.

The term "etchable" and "non-etchable" used above and in the following is not to be taken in the absolute sense of the word but means that the metal in question is one that is not attacked in the etching process in question.

In connection with using chromium, chromium-containing alloys or stainless steel as the water-retaining component which is the most

important kind of planographic process with which the present invention can be used and particular great advantage can be obtained there may be used as is well known copper, brass or bronze as the ink-retaining component. These components will act in the printing process in the said capacities irrespectively whether one or the other is placed in the uppermost position and the present invention can be employed in connection with both possibilities. If chromium or a chromium-containing alloy is placed on a surface of an ink-retaining metal such as copper, brass or bronze it is on the surface of the chromium etc. that the protecting metal is to be placed and the chromium etc. must then be etched through at the same time leaving the protecting metal as a non-etchable metal. An example of an etching agent by means of which this can be carried into effect is hydrochloric acid provided that the protecting metal is one not attacked by this acid for instance lead. If on the other hand an ink-retaining metal such as copper, brass or bronze is placed on the surface of the ink repelling metal, chromium, chromium-containing alloy or stainless steel the ink-retaining metal must now be etchable and an etching agent capable of etching the exposed parts thereof away must be used. Examples of such etching agents are given in the following. Also in this case, however, the protecting metal must be non-etchable to the etching agent used.

According to an embodiment of the invention iron, lead or tin or alloys thereof are used for the protecting metal. These metals are easy to apply in the electrolytical way and they offer an excellent protection for the parts of the metallic interlayer which are not to be removed. Also in this case there may be used an acid etching and if the metallic interlayer is an ink-retaining component such as copper, brass or bronze, chromic acid is very suitable since it removes such metals very readily and does not attack the protecting metals even iron.

According to another embodiment of the invention not only iron, lead or tin but also many other metals may be used for the protecting metal such as zinc or cadmium if for the etching agent there is used a sulphidizing agent such as a solution of an alkali metal sulphide or alkali metal polysulphide, which converts the intermediate metal layer into an easily removable sulphide if this consists of copper, brass or bronze. If it consists of chromium etc. evidently this etching cannot be used.

In case of extremely delicate printing elements this embodiment may be even preferable to the acid-etching method mentioned above since it is practically undamaging to such elements.

If a sulphidizing etching agent is used it is preferable to support the etching process by using an electric current, which is passed through the etching agent using the printing form as one of the electrodes in the circuit. To remove the sulphide formed by the etching process it may be necessary to employ a powerful rinsing or a slight rubbing action.

Generally the protecting metal is to be removed from the surface of the intermediate layer of metal before printing. This can be done by means of an acid etching agent which does not attack either of the two metals entering into the planographic printing process. In most cases diluted sulphuric acid will be found suitable.

The deposition of the protecting metal is pref-

erably carried out by means of the electric current.

Two embodiments of the invention will be described in the following with reference to the drawing in which Figs. 1-4 show schematically the various layers of a printing form in section on four stages of its production.

*Example 1*

A plate S of stainless steel or of copper or nickel coated on one side with chromium or any other plate of which at least one surface is a surface of chromium or chromium-containing alloys, for instance, stainless steel is covered on the surface consisting of chromium, chromium-containing alloy or stainless steel with a continuous layer of copper C. To the layer of copper there is applied a light sensitive film, for example, a chromate-gelatine layer which is then exposed to the influence of light through a transparent positive and developed in the ordinary manner. The parts of the copying layer remaining after development on the surface of the continuous layer of copper is designated by L in Fig. 1.

The printing form appears now as a chromate-colloid image on a base of copper. This image is negative when considered as an image of colloid and positive if it is considered as an image of uncovered copper surfaces.

In order to protect the copper surface elements during the removal of the areas now covered by colloid a protecting metal F is applied to the said areas. The protecting consists in iron which is deposited in the electrolytical way.

For this purpose an aqueous solution of an iron salt is applied to the surface of the plate placed on a table by means of a brush in the bottom of which at the roots of the bristles an iron electrode connected through the handle to the positive pole of a source of electricity is placed. At the same time the printing form is connected to the negative pole. By working on the plate with such a brush a layer of iron is in all parts of sufficient thickness can be deposited in all openings of the layer of colloid even the tiniest.

Then the colloid image is removed by hot water and the plate is now composed as shown in Fig. 2.

Now the copper is removed by etching from the areas which are not covered with iron. The etching agent consists of chromic acid made by dissolving chromic acid anhydride in water. The plate is now composed as shown in Fig. 3.

After this the layer of iron is removed by means of an etching agent consisting of a solution of diluted sulphuric acid or nitric acid after which the plate composed as shown in Fig. 4 is ready of use.

In the drawing the layer of copper and the layer of protecting metal is shown in exaggerated thickness. In fact the layer of copper must be as thin as possible. Theoretically it needs only be of molecular thickness, but to increase its resistance to wear its thickness may practically be increased to, for example, a few hundredths of a millimeter. The protecting metal may be used in similar thickness.

*Example 2*

The plate S is of copper or steel coated on at least one side with a layer of copper. This plate is now covered on the copper surface with a con-

tinuous layer of chromium C, for instance, by electrodeposition. As to the thickness of the layer of chromium the same considerations apply as in the case of copper in Example 1. The copying layer is applied in the same manner as in Example 1 and exposed through a negative.

The printing form shows now a colloid image on a base of chromium. The image is positive when considered as a colloid image and negative if considered as an image of uncovered chromium surface elements.

In order to protect the chromium surface areas to be maintained during etching of the areas to be removed a protecting metal F consisting of lead is deposited on the surface areas not covered by the colloid image. The lead is deposited by electrolysis in the manner described in Example 1. The colloid image is removed and the plate will be of the construction shown in Fig. 2.

Then the chromium is removed from the areas not covered by lead for which purpose the etching agent consists of hydrochloric acid which will not attack the lead and copper. The plate is now constructed as shown in Fig. 3.

Finally the layer of lead is removed by means of nitric acid after which the plate shown in Fig. 4 will be ready for use.

**I claim:**

1. Method of producing a planographic printing form with bimetallic surface comprising the steps of: depositing galvanically on to a base of stainless steel a thin continuous layer of copper, applying to this galvanically deposited layer an image forming coating covering such parts of the layer subsequently to be removed, galvanically depositing on uncovered parts of the copper layer a thin layer of iron, removing the image forming coating, removing uncovered copper down to the base layer by means of chromic acid and removing the iron layer by dilute sulphuric acid.

2. Method of producing a planographic printing form with bimetallic surface comprising applying to the copper layer of a bimetallic printing form consisting of a stainless steel base carrying a thin continuous layer of copper, an image forming coating covering such parts of the copper layer which are subsequently to be removed, depositing galvanically on the uncovered parts of the copper layer a thin layer of iron, removing the image forming coating, removing uncovered copper down to the base layer by means of chromic acid, and then removing the iron resist.

CLAES BØRGE ALLER.

**REFERENCES CITED**

The following references are of record in the file of this patent:

**UNITED STATES PATENTS**

| Number    | Name       | Date           |
|-----------|------------|----------------|
| 444,951   | Goodwin    | Jan. 20, 1891  |
| 758,599   | Sachers    | Apr. 26, 1904  |
| 797,668   | DeJey      | Aug. 22, 1905  |
| 1,376,365 | Wertheimer | Apr. 26, 1921  |
| 1,783,664 | McFarland  | Dec. 2, 1930   |
| 1,871,734 | Trist      | June 23, 1931  |
| 1,886,817 | Johnston   | Nov. 8, 1932   |
| 2,214,950 | Aller      | Sept. 17, 1940 |
| 2,241,585 | Day        | May 13, 1941   |
| 2,408,220 | Lum        | Sept. 24, 1946 |